

# UNITED STATES PATENT OFFICE.

LESLIE CARL DUTRO, OF LONG BEACH, CALIFORNIA.

## OIL CUP.

1,408,180.

Specification of Letters Patent. Patented Feb. 28, 1922.

Application filed October 5, 1920. Serial No. 414,820.

To all whom it may concern:

Be it known that I, LESLIE C. DUTRO, a citizen of the United States, and a resident of Long Beach, in the county of Los Angeles and State of California, have invented a new and Improved Oil Cup, of which the following is a full, clear, and exact description.

This invention relates to improvements in oil cups, and more particularly to oil cups having an automatic feed of oil controlled by the temperature of the bearing.

A further object is to provide an oil feeding device of the character stated, which can be manufactured and sold at an extremely low price, which will feed oil as the bearing increases in temperature and which will automatically cease feeding the oil as the temperature of the bearing falls.

With these and other objects in view the invention consists in certain novel features of construction, and combinations and arrangements of parts as will be more fully hereinafter described and pointed out in the claims.

The accompanying drawing is a view in longitudinal section illustrating my invention.

1 represents my improved oil cup which is provided at its upper end with an inlet nipple 2, the latter externally screw threaded as shown at 3, for the reception of a cap 4 and a gasket 5 to securely close the inlet and render the cup airtight. It is obvious, of course, that the particular form of inlet and the manner of making the same airtight may be varied without departing from my invention.

The closed bottom 6 of the cup 1 is made centrally with an integral well 7, the latter externally screw threaded as shown at 8, and adapted to screw into a threaded opening 9 in a bearing 10. A vertical well outlet tube 11 is secured in the bottom 12 of the well and is open to the bearing and this tube 11 projects upwardly into the well the desired distance.

A cup outlet tube 13 is secured in the bottom of the cup 1 communicating with the interior of the cup and projects downwardly into the well 7.

14 represents the lubricant which is located in the cup 1 and which overflows into the well 7 and from the latter flows into the bearing 10 through the tube 11.

The operation of my improved lubricant cup is entirely automatic. When the cup is filled or partially filled with lubricant, a portion thereof will flow into the well 7, but due to the fact that the cup 1 is airtight, the escape of oil from the cup 1 will cause a partial vacuum to be formed in the upper portion thereof so that the flow of oil will cease under normal conditions. When the temperature of the bearing increases, the heat will be transmitted to the well cup and lubricant to cause an expansion of the lubricant and also an expansion of the air. This expansion will force the lubricant downwardly through the tube 13 into the well 7 and will overflow through the tube 11 into the bearing 10 to cool the latter.

As the temperature decreases, the expansion of the fluid will decrease, and if this decrease in temperature is sufficient, the lubricant will be sucked up from the well 7 through the tube 13 and air will be drawn from the bearing through the tube 11 into the well. The feed of lubricant is, therefore, controlled automatically by the temperature of the bearing and in carrying out this automatic operation, the metal of the cup as well as the lubricant and the air expand and contract in accordance with the temperature of the bearing so that the feed of lubricant is automatically maintained and air is drawn into the well and cup from the bearing to maintain the normal atmospheric pressure within the cup.

The well 7 allows leeway in the operation of the cup. This leeway may be accomplished by extending or shortening the tube 13. By lengthening the tube 13 so that it terminates near the bottom of the well, the well has to be filled up to a point level with the top of the tube 11 before it begins to feed to the bearing, and when a contraction takes place in the well, the liquid is drawn up into the cup until a point level with the bottom of the tube 13 is reached, when direct communication with the atmosphere is made through the tube 11 and the bearing 10 so that the oil in the well is drawn up into the cup.

A further advantage of the enclosed well is that when the cup is jarred or shaken, instead of shaking a few drops directly out into the bearing, they are shaken from the cup into the well and when the balance is established, this excess of lubricant is drawn

# UNITED STATES PATENT OFFICE.

CHARLES S. REEVE, OF GRANTWOOD, NEW JERSEY, ASSIGNOR TO THE BARRETT COMPANY, A CORPORATION OF NEW JERSEY.

## EMULSION AND PROCESS OF MAKING THE SAME.

1,408,224.

Specification of Letters Patent. Patented Feb. 28, 1922.

No Drawing.

Application filed July 23, 1920. Serial No. 398,391.

To all whom it may concern:

Be it known that I, CHARLES S. REEVE, a citizen of the United States, residing at Grantwood, in the county of Bergen and State of New Jersey, have invented certain new and useful Improvements in Emulsions and Processes of Making the Same, of which the following is a specification.

This invention relates to bituminous materials. It relates especially to bituminous materials of a liquid or semi-liquid nature which contain clay or similar material.

The object of the invention is to produce an aqueous emulsion of bituminous materials which shall be more stable than similar emulsions heretofore produced. Another object of the invention is to produce a process by which the bituminous material can be suspended in the aqueous dispersing medium for a longer period than has heretofore been possible with the usual processes.

It has been known for a long time that an emulsion could be produced by mixing clay, water, and bituminous materials and stirring the same, whereupon a certain proportion of the bituminous material and the clay would become permanently suspended in the water and would not settle upon long standing. It has been found for example that when an emulsion of about 4 parts soft coal tar pitch having a melting point of 100°-110° F. (by cube in water method), 3 parts of clay and 3 parts of water were dispersed in 9 parts of water to one part of this emulsion, about 65% by volume of this mixture would remain in suspension at the end of ten minutes. Such emulsions are unsatisfactory, however, because there is a tendency for the materials to settle out upon long standing, and it is also impossible to procure the concentration of bituminous material in the emulsion that is sometimes desirable.

By the present invention a mixture of bituminous material such as asphalt, coal tar, etc., and argilliferous materials such as clay, is made to form an emulsion in water in such a manner that upon dispersion in water a larger percentage of bitumen and clay will be retained in suspension than in the old processes. In order to bring about this result, I have found that when ammonium hydroxide is added to the water the product is very much improved in the respects above mentioned.

In order to make the invention more clearly understood, the following specific example is given for illustrative purposes but it is not intended to restrict the invention to the exact proportions or materials herein mentioned. For example, an emulsion of the same materials and proportions above described may be prepared excepting for the addition of ammonium hydroxide to the amount of about 0.25% of the weight of the emulsion. Upon dispersing this emulsion in 9 parts of water to 1 part of emulsion, it has been found that about 90% by volume of the mixture would remain in suspension at the end of 10 minutes as compared with 65% when the hydroxide was omitted. The proportion of ammonium hydroxide has been varied from about 2/10 of one per cent to forty-five hundredths of one per cent or higher, but no noticeable improvement has been found by using proportions of hydroxide greatly in excess of the latter amount. The proportions of bituminous material and clay may also be varied over a wide range with satisfactory results, since in all cases the addition of the hydroxide tends to make the emulsion more permanent. Although a relatively soft pitch has been described in this specification, I have obtained similar results with harder pitches. I therefore do not desire to limit myself to soft pitch but include any residue obtained by the distillation of tar.

Another advantage of using the hydroxide as set forth in this invention is that it causes a more rapid set or hardening of the composition when it is subjected to a drying operation.

The composition or emulsion produced as above set forth can be used in its fluid or semi-fluid condition as a paint or coating and when so applied, the water dries out and the hydroxide causes the layer to harden quite rapidly. Also, the emulsions which contain no ammonia break down more quickly and readily than those which contain it. So far ammonium hydroxide has given decidedly the most satisfactory results, but sodium hydroxide or potassium hydroxide may be used to some advantage.

I claim:

1. A composition of matter comprising bituminous material, argilliferous material, water and ammonium hydroxide.
2. A composition of matter comprising

pitch, argilliferous material, water and ammonium hydroxide.

3. A composition of matter comprising about 4 parts bituminous material, 3 parts clay, water, and ammonium hydroxide.

4. A composition of matter comprising a mixture of about 4 parts soft coal tar pitch, 3 parts clay, and 3 parts water, containing

between 0.2% and 0.5% by weight of ammonium hydroxide.

5. The process which comprises emulsifying a mixture of bituminous material and clay in water containing ammonium hydroxide.

In testimony whereof I affix my signature. 15  
CHARLES S. REEVE.